

# UNITED STATES PATENT OFFICE.

OSKAR MATTER, OF TROISDORF, GERMANY, ASSIGNOR, BY MESNE ASSIGNMENTS, TO  
THE VEREINIGTE KOLN-BOTTWEILER PULVERFABRIKEN, OF BERLIN, GERMANY.

## INITIAL IGNITER.

1,254,147.

Specification of Letters Patent. Patented Jan. 22, 1918.

Application filed April 17, 1913. Serial No. 761,843.

*To all whom it may concern:*

Be it known that I, OSKAR MATTER, a subject of the Emperor of Germany, and a resident of Troisdorf, in the Empire of Germany, have invented a certain new and useful Improvement in Initial Igniters, and do hereby declare that the following is a full, clear, and exact description thereof.

While my invention comprises an improvement in initial igniters in general, it has special reference to the production of certain types of initial igniters as herein-after set forth.

It has been found in the past that detonators containing fulminate of mercury and certain inorganic substances such, for example, as chlorate of potassium, may be made more powerful by substituting for a part of the fulminate of mercury a quantity of picric acid, trinitrotoluol or tetranitromethylanilin.

I have discovered, however, that even more powerful detonators may be made by the use of nitropentaerythrite, especially if this is used in connection with any detonating substance such as fulminate of mercury or lead azid. The powerful effect of nitropentaerythrite is also, of course, observed in the case where it is used in connection with further detonating substances such, for example, as tetranitromethylanilin, trinitrotoluol, picric acid, etc.

A detonator made in accordance with my invention may, for example, be produced as follows: A detonating composition made in accordance with my invention may be comprised of 1 gram of nitropentaerythrite and a layer of .2 gram of lead azid. It is found that a detonator of this kind gives in a lead cylinder of 10x10 cm. an average net expansion of about 46 ccm., while, on the contrary, a detonator made with 1 gram of tetranitromethylanilin and a layer of .2 gram of lead azid, fired under like conditions, gives an expansion of only 34 ccm. to 35 ccm., and a detonator comprised of 1 gram of trinitrotoluol with a layer of .2 gram of lead azid, similarly fired, gives an expansion of only 29 ccm. to 30 ccm.

Copies of this patent may be obtained for five cents each, by addressing the "Commissioner of Patents, Washington, D. C."

My invention is especially applicable also as a priming for explosives very difficult to detonate such, for example, as crystalline trinitrotoluol containing 10% of castor oil. A charge of 50 grams of trinitrotoluol containing 10% of castor oil fired with the nitropentaerythrite lead azid detonator given above, in a conical lead cylinder of 400 mm. diameter, gives an average expansion of 1365 ccm.

My invention is also particularly suitable when applied as a priming for projectile bursting charges. An initial igniter made in accordance with my invention possesses great detonation safety and is absolutely insensitive to external influences such as heat, moisture, etc.

While I have described my invention above in detail, I wish it to be understood that many changes may be made therein without departing from the spirit of my invention.

I claim:

1. An initial igniter composition containing nitropentaerythrite and another detonating substance. 75
2. An initial igniter composition containing nitropentaerythrite and lead azid.
3. An initial igniter composition containing nitropentaerythrite and a layer of another detonating substance. 80
4. An initial igniter composition containing nitropentaerythrite and a layer of lead azid.
5. A detonator comprising nitropentaerythrite and another detonating substance. 85
6. A detonator comprising nitropentaerythrite and lead azid.
7. A detonator comprising nitropentaerythrite and a layer of another detonating substance. 90
8. A detonator comprising nitropentaerythrite and a layer of lead azid.

In testimony that I claim the foregoing I have hereunto set my hand.

OSKAR MATTER.

Witnesses:

LOUIS VANDORY,  
MARIA PALMEN.